# EUROPEAN PATENT SPECIFICATION

(11) **EP 1 964 952 B1**
(45) Date of publication and mention of the grant of the patent: **01.06.2011**
(21) Application number: 08151814.4
(22) Date of filing: 22.02.2008
(51) Int. Cl.: D02G 3/38, D02G 3/44

(54) **Yarn for technical fabrics and method for manufacturing the same**
Garn für technische Fasern und Verfahren zu seiner Herstellung
Fil pour tissus techniques et son procédé de fabrication

(30) Priority: 28.02.2007 IT BS20070027
(43) Date of publication of application: 03.09.2008
(73) Proprietor: Filtes International S.r.l., 25031 Capriolo (BS) (IT)
(72) Inventor: Carrara, Sergio, 24067 Sarnico (Bergamo) (IT)
(74) Representative: Pulieri, Gianluca Antonio

(56) References cited:
- US-A- 5 845 476
- US-A1- 2004 148 921
- US-A1- 2005 086 924
- US-B1- 6 279 305
- US-B1- 6 467 251
- US-B1- 6 779 330

## Description

The present invention relates to a yarn for protective fabrics, i.e. a yarn having high wear resistance mechanical properties, usually called a "technical" yarn in the field, which is suitable for making fabrics for manufacturing work gloves and other safety garments.

A number of technical yarn types are available.

US 4.777.789, for example, illustrates a yarn consisting of an inner core made of a monofilament or multifilament, such as of glassfiber, on which an inner thread is wound, for example made of stainless steel. The core and the inner thread are covered by a first thread wound in a first winding direction, which forms a first covering layer; the first covering layer is covered by a second thread wound in a second winding direction, which forms a second covering layer. The first wound thread and the second wound thread are made of, for example, aramide resin.

Some examples of yarns are disclosed in US 2005/086924, US 6,467,251, US 5,845,476, US 6,279,305, US 6,779,330 e US 2004/148921.

Moreover, US 4,202,382, US 3,726,078, EP-A2-0125505, US 4,470,251, US 4,158,946, US 3,336,744 further illustrate other types of yarns.

The object of the present invention is to provide a novel type of yarn, having high mechanical characteristics, even more suitable to make technical fabrics as compared with known yarns, especially for protective garments.

Particularly, the yarn being the object of the present invention exhibits a high cut strength and a high workability during garment weaving.

This object is achieved by a yarn in accordance with claim 1, which can be obtained by means of the fabrication methods in accordance with claims 25 and 26.

The characteristics and advantages of the yarn and method according to the present invention will be apparent from the description given below, which is given by way of a non-limiting example, in accordance with the figures below, in which:

Fig. 1 to 5 illustrate variant embodiments of a yarn according to the present invention; and

Fig. 6 illustrates a garment made by means of the yarn of the present invention, for example, a glove.

With reference to Fig. 1, with 1 has been generally designated a yarn comprising a core consisting of a continuous filament 2.

The continuous filament 2 consists of a monofilament, such as made of glass or an elastic material, for example Lycra®, extending along a filament axis X.

For example, the filament 2 has linear density of 110 dtex.

The yarn 1 further comprises a first thread 4, wound around the continuous filament 2, such as to provide a first covering of the latter, in contact with the outer surface of the filament.

The first thread 4 is wound around the filament 2 in a first winding direction and with an inclination relative to the filament axis X. For example, the first thread is wound on the filament such as to obtain 500 coils along one linear meter of filament.

Preferably, the first thread is a polyester or polyamide continuous filament.

Preferably, the first thread 4 is further worked on the surface thereof such as to have a high roughness.

For example, the first thread has a linear density ranging between 50 and 200 dtex, preferably of 110 dtex.

The first cover provides a continuous layer, which covers the filament 2, since the coils of the first thread 4 wound on the filament 2 are axially tangential relative to each other, such as to avoid leaving gaps therebetween, from which the underlying filament 2 may appear. In other words, the first thread forms a closed coiling.

The yarn 1 further comprises a second thread 6 wound around the first cover, such as to provide a second cover thereon.

The second thread 6 is wound around the first cover in a second winding direction, opposite the first one. For example, the second thread has an inclination relative to the filament axis X opposite the first thread inclination.

For example, the second thread is wound on the first cover such as to obtain 500 coils along a linear meter.

Preferably, the second thread is a polyester or polyamide continuous filament.

Preferably, the second thread 6 is further worked on the surface thereof such as to have a high roughness.

For example, the second thread has a linear density ranging between 50 and 200 dtex, preferably of 110 dtex.

Preferably, the linear density of the second thread is equal to the linear density of the first thread.

The second cover provides a continuous layer that covers the first cover because the coils of the second thread are axially tangential to each other, such as to avoid leaving gaps therebetween, from which the first underlying cover may appear.

Furthermore, the yarn 1 comprises a third thread 8, wound on the second cover.

The third thread 8 does not provide a continuous covering on the second cover, since the twisting is carried out such that a gap is left between the coils, in order to make the second underlying cover visible and accessible. In other words, the third thread forms an open coiling, as it is wound on the covered thread.

For example, the third thread has a twisting with a twist linear density between 100 and 200 per linear meter, preferably equal to 170 twists per linear meter.

Preferably, the third thread 8 is wound around the second cover according to a twisting direction opposite that of the second thread.

The third thread is a high-tenacity yarn, i.e. with a tenacity ranging between 40 and 120 cN/tex, preferably of 70 cN/tex.

Preferably, the third thread is made of a high-tenacity primary organic matrix (generally having tenacity values of 1.5 to 3.5 N/tex), coupled to further fibers.

For example, the third thread is made as a yarn, for example by means of ring spinning, from discontinuous polyethylene fibers and polyamide fibers, for example at the same or different weight ratio.

For example, the third thread is made as a yarn from discontinuous Dyneema® fibers and polyamide.

Fig. 2 illustrates a further variant embodiment of the yarn according to the present invention.

In Fig. 2, and following figures, the same numerals in Fig. 1 are used to designate similar parts.

According to the variant embodiment illustrated herein, the yarn 1 comprises a multifilament core, such as consisting of two filaments 2a, 2b, parallel to each other.

Similarly to the variant embodiment in Fig. 1, the core is covered by the first cover being the first thread 4, by the second cover formed being the second thread 6, and twisted along with the third thread 8.

Fig. 3 illustrates a further embodiment of the yarn according to the present invention.

According to the variant embodiment illustrated herein, the yarn 1 comprises a monofilament core, consisting of an individual filament 2, covered by the first cover being the first thread 4, which is, in turn, covered by the second cover being the second thread 6, on which a third thread 8a and a fourth thread 8b are twisted.

The fourth thread 8b has structural characteristics similar to those of third thread 8a.

For example, the third thread 8a has a first twisting direction, such as opposite that of second thread 6, and the fourth thread 8b has a second twisting direction, equal to the first twisting direction.

It will be understood that, in the embodiments described above, the first cover is in direct contact with the yarn core; in other words, there are no intermediate threads between the glassfiber core and the first cover.

Fig. 4 illustrates a further embodiment of the yarn according to the present invention.

According to the embodiment illustrated herein, the yarn comprises a multifilament core, for example consisting of two continuous filaments 2a, 2b parallel to each other, on which a coupling thread 10 is twisted.

On the coupling thread 10 is wound the first thread 4 of the first cover, on which is wound the second thread 6 of the second cover, on which are twisted the third thread 8a and the fourth thread 8b, or, in a further embodiment, an individual third thread 8.

Fig. 5 illustrates a further embodiment of the yarn according to the present invention.

According to the embodiment illustrated herein, the yarn comprises a monofilament core, consisting of an individual filament 2, on which the coupling thread 10 is twisted.

On the coupling thread 10 is wound the first thread 4 of the first cover, on which is wound the second thread 6 of the second cover, on which is twisted the third thread 8, or, in a still further embodiment, the third thread 8a and the fourth thread 8b.

According to other embodiments, the third and/or the fourth thread, according to embodiments here above, comprises, besides a stiff yarn, for example from discontinuous polyethylene fibers and polyamide fibers, also a flexible yarn, for example a synthetic polyurethane fiber, for example lycra®.

For example, the third thread is made as a yarn from discontinuous Dyneema® fibers and polyamide.

The yarn according to the present invention is particularly suitable to make technical fabrics for protective garments, such as a glove 100.

The yarn according to the present invention can be fabricated according to a fabrication method comprising the steps of:

- arranging at least one glass continuous filament;

- feeding the continuous filament along a filament axis (X);

- wounding a first thread around the continuous filament being fed, thus providing a first cover overlapping the continuous filament with closed coiling, said winding being carried out according to a first winding direction;

- winding a second thread around the first cover already wound around the continuous filament, thus providing a second cover overlapping the first cover with closed coiling, said second cover having a second winding direction, opposite the first one;

- twisting a third thread (8) around the second cover already wound on the first cover, with open coiling in a twisting direction opposite that of second cover.

Particularly, the yarn according to the variant embodiment in Fig. 3 can be fabricated according to a fabrication method comprising the steps of:

- arranging at least one continuous filament;

- feeding the continuous filament along a filament axis X;

- winding a first thread around the continuous filament being fed, thus providing a first cover overlapping the continuous filament with closed coiling, said winding being provided according to a first winding direction;

- winding a second thread around the first cover already wound around the continuous filament, thus providing a second cover overlapping the first cover with closed coiling, said second cover having a second winding direction, opposite the first one;

- feeding the covered thread along with a third thread and a fourth thread;

- twisting the covered thread along with the third thread and the fourth thread, such that the third thread and fourth thread form an open coiling in the twisting direction opposite that of second cover.

It has been innovatively found how the yarn according to the present invention has excellent mechanical characteristics and a high workability for fabricating technical fabrics.

Particularly, it has been found how the third thread overlapping with open coiling the second cover provides the yarn with a high cut strength, without depriving the fabric of the softness required to make a comfortable garment.

It is believed that the increase in the cut strength is due to the holding action applied by the third thread on the coils of the second cover.

In other words, when a cutting body cuts the fabric made of the yarn according to the present invention, this cut presumably causes a local rupture of the second cover, which, however, does not flake off, due to the holding action applied by the third thread wound thereon.

In confirmation of this unexpected result, laboratory tests have been carried out, and particularly those tests pursuant to rule EN 388/03 (2003 ed.), which assigns level 5 to a fabric resisting to shear after twenty test cycles (Chapt. 6.2 of the rule) and level 4 to a fabric resisting to abrasion after eight thousand cycles (Chapt. 6.1 of the rule).

The fabric made of the yarn of the present invention has achieved level 5 cut resistance, and level 4 abrasion resistance.

According to a still further advantageous aspect, contrary to present knowledge, the provision of a third thread twisted on the second cover increases the fabric softness.

It is believed that this advantageous and unexpected effect is due to the fact that the third thread provides such a relief that, when the yarns are mutually engaged within the weft of a fabric, these are rested on each other at this relief. This increases the tendency of the yarn to flexibility and thus the fabric softness.

In other words, it is believed that this advantageous and unexpected effect is due to a reduced contact surface between the weft yarns of a fabric, which is due to the provision of the third externally-twisted thread.

Advantageously, furthermore, the provision of two threads twisted to the covered thread, in the same twisting direction, provides the fabric with a particular cut strength and abrasion resistance, while maintaining the fabric softness.

To opposite twisting directions, in fact, would correspond an undesired stiffening of the fabric.

According to a further advantageous aspect, the provision of the first and second covers provides the yarn with the desired strength for high-performing technical fabrics, while, by suitably selecting the materials, the fabric is sufficiently soft to provide a comfortable garment, or the mechanical properties can be changed as desired.

Advantageously, furthermore, the first and/or second threads have a surface roughness suitable to create a good grip of the first cover to the glass filament and/or the second cover to the first cover.

It is understood that those skilled in the art may carry out variations and modifications to the yarn and method described above, which are however all contemplated within the scope of protection as defined in the following claims.

## Claims

1. A yarn (1) comprising:
- a core comprising at least one continuous filament (2) extending along a Filament axis (X);
- a first thread (4) wound around the filament (2) along said filament axis (X) thus forming a first closed-coiling cover, said first thread being wound in a first winding direction;
- a second thread (6) wound about the first cover along said filament axis forming a second closed-coiling cover, said second thread being wound in a winding direction opposite the winding direction of the first thread;
**characterized in that**
- a third thread (8) is wound around the second cover along the filament axis, twisted with an open coiling; whereby
the third thread is a high-tenacity yam, i.e. having a tenacity ranging between 40 and 120 cN/tex.

2. A yam according to claim 1, wherein the third thread is wound such that the coils are axially spaced from each other, thus providing said open coiling.

3. A yarn according to claim 1 or 2, wherein the third thread is a yarn having a tenacity of 70 cN/tex.

4. A yam according to any of the previous claims, wherein the third thread (8) is a polyethylene and polyamide discontinuous fiber yam.

5. A yam according to any of the previous claims, wherein the third thread is a polyethylene and polyamide discontinuous fiber yam at either the same or different weight ratio.

6. A yarn according to any preceding claim, wherein the third thread (8) is twisted in a twisting direction opposite the winding direction of the second thread (6).

7. A yam according to any preceding claim, further comprising a fourth thread, twisted with an open coiling on the third thread.

8. A yarn according to claim 7, wherein the fourth thread has the same twisting direction of the third thread.

9. A yam according to claim 7 or 8, wherein the fourth thread is a high-tenacity yam.

10. A yarn according to any preceding claim, wherein the coils of the first and second covers are axially in contact with each other, thus providing said closed coiling.

11. A yam according to any preceding claim, wherein the first thread is a polyester or polyamide continuous filament.

12. A yam according to any preceding claim, wherein the second thread is a polyester or polyamide continuous filament.

13. A yam according to any preceding claim, wherein the first thread has a linear density of 50 to 200 dtex.

14. A yam according to claim 13, wherein the first thread has a linear density of 110 dtex.

15. A yarn according to any preceding claim, wherein the second thread has a linear density of 50 to 200 dtex.

16. A yarn according to claim 15, wherein the second thread has a linear density of 110 dtex.

17. A yam according to any preceding claim, wherein the filament (2) is made of glass.

18. A yam according to any claim 1 to 16, wherein the filament (2) is made of elastic material, such as Lycra®.

19. A yarn according to any preceding claim, wherein the filament has a linear density of 100 to 120 dtex.

20. A yarn according to claim 19, wherein the filament (2) has a linear density of 110 dtex.

21. A yam according to any preceding claim, wherein the core comprises two parallel continuous filaments (2a, 2b).

22. A yam according to any preceding claim, wherein the core comprises a coupling thread (10) wound with an open coiling, arranged between the filament and the first cover.

23. A fabric comprising a yam made in accordance with any preceding claim.

24. A garment comprising a fabric according to claim 23.

25. A method for fabricating a yarn comprising the steps of:
- arranging at least one continuous filament (2);
- feeding the continuous filament along a filament axis (X);
- wounding a first thread (4) around the continuous filament being fed, thus providing a first cover overlapping the continuous filament with closed coiling, said winding being carried out according to a first winding direction;
- winding a second thread (6) around the first cover already wound around the continuous filament, thus providing a second cover overlapped to the first cover with closed coiling, said second cover having a second winding direction, opposite the first one;
- twisting a third thread (8) around the second cover already wound on the first cover, with open coiling in a twisting direction opposite that of second thread (6), said third thread being a high-tenacity yarn, i.e. having a tenacity ranging between 40 and 120 cN/tex.

26. A method for fabricating a yam comprising the steps of:
- arranging at least one continuous filament;
- feeding the continuous filament along a filament axis (X);
- winding a first thread around the continuous filament being fed, thus providing a first cover overlapping the continuous filament with closed coiling, said winding being provided according to a first winding direction;
- winding a second thread around the first cover already wound around the continuous filament, thus providing a second cover overlapping the first cover with closed coiling, said second cover having a second winding direction, opposite the first one;
- feeding this covered thread along with a third thread and a fourth thread;
twisting the covered thread along with the third thread and the fourth thread, such that the third thread and fourth thread form an open coiling in the twisting direction opposite that of second cover, said third thread being a high-tenacity yam, i.e. having a tenacity ranging between 40 and 120 cN/tex.

27. A yam according to any one of claims 1-22, wherein the third and/or the fourth thread comprises, besides a stiff yam, for example from discontinuous polyethylene fibers and polyamide fibers, also a flexible yam, for example a synthetic polyurethane fiber.

## Patentansprüche

1. Garn enthaltend:
- einen Kern mit wenigstens einem fortlaufenden Filament (2), das sich entlang einer Filamentachse (X) erstreckt;
- einen ersten Faden (4), der um das Filament (2) herum entlang der genannten Filamentachse (X) gewickelt ist und so eine erste Ummantelung in Form einer geschlossenen Wicklung bildet, wobei der genannte erste Faden in einer ersten Wickelrichtung gewickelt ist;
- einen zweiten Faden (6), der um die erste Ummantelung entlang der genannten Filamentachse gewickelt ist und eine zweite Ummantelung in Form einer geschlossenen Wicklung bildet, wobei der genannte zweite Faden in einer entgegen der Wickelrichtung des ersten Fadens verlaufenden Richtung gewickelt ist;
**dadurch gekennzeichnet dass** ein dritter Faden (8) um die zweite Ummantelung entlang der Filamentachse gewickelt ist und zwar gewickelt in Form einer offenen Wicklung, wobei es sich bei dem dritten Faden um ein hochfestes Garn handelt, d.h. es weist eine Festigkeit von 40 bis 120 cN/tex auf.

2. Garn nach Anspruch 1, wobei der dritte Faden so gewickelt ist, dass die einzelnen Windungen in einem axialen Abstand voneinander verlaufen und so die genannte offene Wicklung bilden.

3. Garn nach Anspruch 1 oder 2, wobei der dritte Faden ein Garn mit einer Festigkeit von 70 cN/tex darstellt.

4. Garn nach einem der vorhergehenden Ansprüche, wobei der dritte Faden (8) ein diskontinuierliches Polyethylen- und Polyamid-Fasergarn ist.

5. Garn nach einem der vorhergehenden Ansprüche, wobei der dritte Faden (8) ein diskontinuierliches Polyethylen- und Polyamid-Fasergarn mit entweder dem gleichen oder einem unterschiedlichen Gewichtsverhältnis ist.

6. Garn nach einem der vorhergehenden Ansprüche, wobei der dritte Faden (8) in einer Richtung gewickelt ist, die sich entgegengesetzt der Wickelrichtung des zweiten Fadens (6) erstreckt.

7. Garn nach einem der vorhergehenden Ansprüche, das weiterhin einen vierten Faden aufweist, der mit einer offenen Wicklung auf den dritten Faden gewickelt ist.

8. Garn nach Anspruch 7, wobei der vierte Faden die gleiche Wickelrichtung aufweist wie der dritte Faden.

9. Garn nach Anspruch 7 oder 8, wobei es sich bei dem vierten Faden um ein hochfestes Garn handelt.

10. Garn nach einem der vorhergehenden Ansprüche, wobei die Wicklungen der ersten und der zweiten Ummantelung sich in axialem Kontakt miteinander befinden und so die geschlossene Wicklung bilden.

11. Garn nach einem der vorhergehenden Ansprüche, wobei der erste Faden (4) ein kontinuierliches Polyester- oder Polyamid-Filament ist.

12. Garn nach einem der vorhergehenden Ansprüche, wobei der zweite Faden (6) ein kontinuierliches Polyester- oder Polyamid-Filament ist.

13. Garn nach einem der vorhergehenden Ansprüche, wobei der erste Faden (4) eine Fadenstärke von 50 bis 200 dtex aufweist.

14. Garn nach Anspruch 13, wobei der erste Faden (4) eine Fadenstärke von 110 dtex aufweist.

15. Garn nach einem der vorhergehenden Ansprüche, wobei der zweite Faden (6) eine Fadenstärke von 50 bis 200 dtex aufweist.

16. Garn nach Anspruch 15, wobei der zweite Faden (6) eine Fadenstärke von 110 dtex aufweist.

17. Garn nach einem der vorhergehenden Ansprüche, wobei das Filament (2) aus Glas besteht.

18. Garn nach einem der Ansprüche 1 bis 16, wobei das Filament (2) aus einem elastischen Material, wie z.B. Lycra®, besteht.

19. Garn nach einem der vorhergehenden Ansprüche, wobei das Filament (2) eine Faserstärke von 100 bis 120 dtex aufweist.

20. Garn nach Anspruch 19, wobei das Filament (2) eine Fadenstärke von 110 dtex aufweist.

21. Garn nach einem der vorhergehenden Ansprüche, wobei der Kern zwei parallele, kontinuierliche Filamente (2a, 2b) aufweist.

22. Garn nach einem der vorhergehenden Ansprüche, wobei der Kern einen Verbindungsfaden (10) aufweist, der in Form einer offenen Wicklung gewickelt ist, die zwischen dem Filament (2) und der ersten Ummantelung angeordnet ist.

23. Gewebe, das ein gemäß irgendeinem der vorhergehenden Ansprüche hergestelltes Garn aufweist.

24. Kleidungsstück, das ein Gewebe nach Anspruch 23 aufweist.

25. Verfahren zur Herstellung eines Garns mit den folgenden Verfahrensschritten:
- Anordnung wenigstens eines kontinuierlichen Filaments (2);
- Zuführung des kontinuierlichen Filaments (2) entlang der Filamentachse (X);
- Wickleln eines ersten Fadens (4) um das zugeführte kontinuierliche Filament, wodurch eine erste Ummantelung bereitgestellt wird, die das kontinuierliche Filament (2) mit der geschlossenen Wicklung überdeckt, wobei die genannte Wicklung gemäß der ersten Wickelrichtung durchgeführt wird;
- Wickeln eines zweiten Fadens (6) um die erste Ummantelung, die bereits über das kontinuierliche Filament (2) gewickelt worden war, wobei eine zweite Ummantelung bereitgestellt wird, die die erste Ummantelung mit der geschlossenen Wicklung überdeckt, wobei die genannte zweite Ummantelung sich in einer zweiten Wickelrichtung erstreckt, die der ersten entgegenläuft;
- Wickeln eines dritten Fadens (8) um die zweite bereits um die erste Ummantelung gewickelte Ummantelung, wobei sich die offene Wicklung in einer Wickelrichtung erstreckt, die der des zweiten Fadens (6) entgegenläuft, wobei es sich bei dem genannten dritten Faden um ein hochfestes Garn handelt, d.h. eine Festigkeit zwischen 40 und 120 cN/tex aufweist.

26. Verfahren zur Herstellung eines Garns mit den folgenden Verfahrensschritten:
- Anordnung wenigstens eines kontinuierlichen Filaments (2);
- Zuführung des kontinuierlichen Filaments entlang der Filamentachse (X);
- Wickeln eines ersten Fadens (4) um das zugeführte kontinuierliche Filament, wodurch eine erste Ummantelung bereitgestellt wird, die das kontinuierliche Filament mit der geschlossen Wicklung überdeckt, wobei die genannte Wicklung gemäß der ersten Wickelrichtung durchgeführt wird;
- Wickeln eines zweiten Fadens (6) um die erste Ummantelung, die bereits über das kontinuierliche Filament gewickelt worden war, wobei eine zweite Ummantelung bereitgestellt wird, die die erste Ummantelung mit der geschlossenen Wicklung überdeckt, wobei die genannte zweite Ummantelung sich in einer zweiten Wickelrichtung erstreckt, die der ersten entgegenläuft;
- Zuführen dieses ummantelten Fadens zusammen mit einem dritten Faden (8) und einem vierten Faden;
- Wickeln des ummantelten Fadens zusammen mit dem dritten Faden (8) und dem vierten Faden in der Weise, dass der dritte Faden und der vierte Faden eine offene Wicklung bilden und zwar in einer Wickelrichtung, die der der zweiten Ummantelung entgegenläuft, wobei es sich bei dem dritten Faden um ein hochfestes Garn handelt, d.h. eine Festigkeit zwischen 40 und 120 cN/tex aufweist.

27. Garn nach einem der Ansprüche 1 bis 22, wobei der dritte und/oder der vierte Faden, abgesehen von einem steifen Garn, zum Beispiel aus diskontinuierlichen Polyethylen-Fasern und Polyamid-Fasern, auch ein flexibles Garn, zum Beispiel eine synthetische Polyurethan-Faser, aufweist.

## Revendications

1. Filé (1) comprenant:
- une âme comprenant au moins un filament continu (2) s'étendant le long d'un axe de filament (X);
- un premier fil (4) enroulé autour du filament (2) le long dudit axe de filament (X) formant ainsi un premier recouvrement à spires jointives, ledit premier fil ayant été enroulé selon une première direction d'enroulement;
- un deuxième fil (6) enroulé autour du premier recouvrement le long dudit axe de filament formant un deuxième recouvrement à spires jointives, ledit deuxième fil étant enroulé dans une direction d'enroulement opposée à la direction d'enroulement du premier fil; **caractérisé en ce qu'**un troisième fil (8) est enroulé autour du deuxième recouvrement le long de l'axe de filament, torsadé en spires non jointives; moyennant quoi le troisième fil est un fil à haute ténacité, c'est-à-dire ayant une ténacité comprise entre 40 et 120 cN/tex.

2. Filé selon la revendication 1, dans lequel le troisième fil est enroulé de sorte que les spires sont axialement espacées les unes des autres, fournissant ainsi lesdites spires non jointives.

3. Filé selon la revendication 1 ou 2, dans lequel le troisième fil est un fil ayant une ténacité de 70 cN/tex.

4. Filé selon l'une quelconque des revendications précédentes, dans lequel le troisième fil (8) est un fil de fibres discontinues de polyéthylène et de polyamide.

5. Filé selon l'une quelconque des revendications précédentes, dans lequel le troisième fil est un fil de fibres discontinues de polyéthylène et de polyamide selon un rapport de poids identique ou différent.

6. Filé selon l'une quelconque des revendications précédentes, dans lequel le troisième fil (8) est torsadé dans une direction de torsion opposée à la direction d'enroulement du deuxième fil (6).

7. Filé selon l'une quelconque des revendications précédentes, comprenant en outre un quatrième fil, torsadé avec des spires non jointives sur le troisième fil.

8. Filé selon la revendication 7, dans lequel le quatrième fil a la même direction de torsion que le troisième fil.

9. Filé selon la revendication 7 ou 8, dans lequel le quatrième fil est un fil à haute ténacité.

10. Filé selon l'une quelconque des revendications précédentes, dans lequel les spires des premier et deuxième recouvrements sont axialement en contact entre eux, fournissant ainsi lesdites spires jointives.

11. Filé selon l'une quelconque des revendications précédentes, dans lequel le premier fil est un filament continu de polyester ou de polyamide.

12. Filé selon l'une quelconque des revendications précédentes, dans lequel le deuxième fil est un filament continu de polyester ou de polyamide.

13. Filé selon l'une quelconque des revendications précédentes, dans lequel le premier fil a une densité linéaire de 50 à 200 dtex.

14. Filé selon la revendication 13, dans lequel le premier fil a une densité linéaire de 110 dtex.

15. Filé selon l'une quelconque des revendications précédentes, dans lequel le deuxième fil a une densité linéaire de 50 à 200 dtex.

16. Filé selon la revendication 15, dans lequel le deuxième fil a une densité linéaire de 110 dtex.

17. Filé selon l'une quelconque des revendications précédentes, dans lequel le filament (2) est réalisé à partir de verre.

18. Filé selon l'une quelconque des revendications 1 à 16, dans lequel le filament (2) est réalisé avec un matériau élastique, tel que le Lycra®.

19. Filé selon l'une quelconque des revendications précédentes, dans lequel le filament a une densité linéaire de 100 à 120 dtex.

20. Filé selon la revendication 19, dans lequel le filament (2) a une densité linéaire de 110 dtex.

21. Filé selon l'une quelconque des revendications précédentes, dans lequel l'âme comprend deux filaments continus parallèles (2a, 2b).

22. Filé selon l'une quelconque des revendications précédentes, dans lequel l'âme comprend un fil de couplage (10) enroulé avec des spires non jointives, agencé entre le filament et le premier recouvrement.

23. Tissu comprenant un fil réalisé selon l'une quelconque des revendications précédentes.

24. Vêtement comprenant un tissu selon la revendication 23.

25. Procédé pour fabriquer un fil comprenant les étapes consistant à:
- agencer au moins un filament continu (2);
- alimenter le filament continu le long d'un axe de filament (X);
- enrouler un premier fil (4) autour du filament continu qui est alimenté, fournissant ainsi un premier recouvrement recouvrant le filament continu avec des spires jointives, ledit enroulement étant réalisé selon une première direction d'enroulement;
- enrouler un deuxième fil (6) autour du premier recouvrement déjà enroulé autour du filament continu, fournissant ainsi un deuxième recouvrement superposé sur le premier recouvrement avec des spires jointives, ledit deuxième recouvrement ayant une deuxième direction d'enroulement opposée à la première;
- torsader un troisième fil (8) autour du deuxième recouvrement déjà enroulé sur le premier recouvrement, avec des spires non jointives dans une direction de torsion opposée à celle du deuxième fil (6), ledit troisième fil étant un fil à haute ténacité, c'est-à-dire ayant une ténacité comprise entre 40 et 120 cN/tex.

26. Procédé pour fabriquer un fil comprenant les étapes consistant à:
- agencer au moins un filament continu;
- alimenter le filament continu le long d'un axe de filament (X);
- enrouler un premier fil autour du filament continu qui est alimenté, fournissant ainsi un premier recouvrement recouvrant le filament continu avec des spires jointives, ledit enroulement étant prévu selon une première direction d'enroulement;
- enrouler un deuxième fil autour du premier recouvrement déjà enroulé autour du filament continu, fournissant ainsi un deuxième recouvrement superposé sur le premier recouvrement avec des spires jointives, ledit deuxième recouvrement ayant une deuxième direction d'enroulement, opposée à la première;
- alimenter ce fil recouvert conjointement à un troisième fil et à un quatrième fil;
- torsader le fil recouvert conjointement au troisième fil et au quatrième fil, de sorte que le troisième fil et le quatrième fil forment des spires non jointives dans la direction de torsion opposée à celle du deuxième recouvrement, ledit troisième fil étant un fil à haute ténacité, c'est-à-dire ayant une ténacité comprise entre 40 et 120 cN/tex.

27. Filé selon l'une quelconque des revendications 1 à 22, dans lequel le troisième et/ou le quatrième fil comprennent, en plus d'un filé rigide, par exemple à partir de fibres de polyéthylène et de fibres de polyamide discontinues, également un filé souple, par exemple une fibre de polyuréthane synthétique.
